



US010233522B2

(12) **United States Patent**  
**Stewart**

(10) **Patent No.:** **US 10,233,522 B2**  
(b4) **Date of Patent:** **Mar. 19, 2019**

(54) **LOW COBALT HARD FACING ALLOY**(71) Applicant: **ROLLS-ROYCE plc**, London (GB)(72) Inventor: **David A Stewart**, Derby (GB)(73) Assignee: **ROLLS-ROYCE plc**, London (GB)

(\*) Notice: Subject to any disclaimer, the term of this patent is extended or adjusted under 35 U.S.C. 154(b) by 114 days.

(21) Appl. No.: **15/400,847**(22) Filed: **Jan. 6, 2017**(65) **Prior Publication Data**

US 2017/0218491 A1 Aug. 3, 2017

(30) **Foreign Application Priority Data**

Feb. 1, 2016 (GB) ..... 1601764.2

(51) **Int. Cl.**

**C22C 38/00** (2006.01)  
**C22C 38/04** (2006.01)  
**C22C 38/34** (2006.01)  
**C22C 38/44** (2006.01)  
**C22C 38/46** (2006.01)  
**C22C 38/48** (2006.01)  
**C22C 38/50** (2006.01)  
**C22C 38/52** (2006.01)  
**C22C 38/56** (2006.01)

(52) **U.S. Cl.**

CPC ..... **C22C 38/56** (2013.01); **C22C 38/001** (2013.01); **C22C 38/002** (2013.01); **C22C 38/04** (2013.01); **C22C 38/34** (2013.01); **C22C 38/44** (2013.01); **C22C 38/46** (2013.01); **C22C 38/48** (2013.01); **C22C 38/50** (2013.01); **C22C 38/52** (2013.01)

(58) **Field of Classification Search**

CPC ..... C22C 38/001; C22C 38/002; C22C 38/04; C22C 38/34; C22C 38/44; C22C 38/46; C22C 38/48; C22C 38/50; C22C 38/52; C22C 38/56

See application file for complete search history.

(56) **References Cited**

## U.S. PATENT DOCUMENTS

2,416,515 A 2/1947 Evans, Jr.  
4,077,801 A \* 3/1978 Heyer ..... C22C 19/055  
148/427  
4,141,762 A \* 2/1979 Yamaguchi et al.  
4,812,177 A \* 3/1989 Maehara ..... C21D 8/005  
148/505  
4,854,185 A \* 8/1989 Lichtenberg ..... F16C 1/226  
188/196 B  
4,981,647 A \* 1/1991 Rothman ..... C22C 30/00  
420/43  
5,077,006 A 12/1991 Culling ..... C22C 38/52  
5,310,431 A \* 5/1994 Buck ..... C22C 38/52  
148/325  
5,512,237 A \* 4/1996 Stigenberg ..... C22C 38/42  
420/38

5,514,328 A \* 5/1996 Menon ..... C22C 38/52  
420/36  
5,660,939 A 8/1997 Burdett ..... C22C 30/00  
148/442  
5,820,817 A \* 10/1998 Angeliu ..... C22C 38/002  
420/40  
5,944,922 A \* 8/1999 Kadoya ..... C21D 6/004  
148/325  
RE36,382 E \* 11/1999 Hultin-Stigenberg ..... C22C 38/42  
420/38  
6,165,627 A \* 12/2000 Miyazaki ..... C22C 38/105  
148/320  
6,174,385 B1 \* 1/2001 Morinaga ..... C22C 38/00  
148/325  
6,426,038 B1 \* 7/2002 Fedchun ..... C22C 38/002  
420/104  
6,426,040 B1 \* 7/2002 Fedchun ..... C22C 38/002  
420/104  
6,464,804 B2 \* 10/2002 Goecmen ..... C21D 6/004  
148/325  
6,479,013 B1 \* 11/2002 Sera ..... B22D 17/2023  
148/325  
6,485,679 B1 \* 11/2002 Sundstrom ..... C22C 38/44  
420/38  
6,630,103 B2 \* 10/2003 Martin ..... C21D 6/02  
148/325

(Continued)

## FOREIGN PATENT DOCUMENTS

|    |              |         |
|----|--------------|---------|
| EP | 0 735 155 A1 | 10/1996 |
| GB | 2 167 088 A  | 5/1986  |
| JP | H06-170584 A | 6/1994  |

## OTHER PUBLICATIONS

Aug. 9, 2017 Search Report issued in European Patent Application No. 17 15 0537.

Oct. 5, 2016 Search Report issued in British Patent Application No. 1601764.2.

(Primary Examiner — Cam N. Nguyen)

(74) **Attorney, Agent, or Firm:** Oliff PLC(57) **ABSTRACT**

A stainless steel alloy comprising essentially of 19 to 22 percent by weight chromium, 8.5 to 10.5 percent by weight nickel, 5.25 to 5.75 percent by weight silicon, 0.25 to 2.0 percent by weight carbon, 4.0 to 10.5 percent by weight molybdenum, 0.3 to 0.5 percent by weight titanium, 0.1 to 0.5 by weight percent nitrogen and the balance iron plus impurities. The impurities may consist of 0 to 0.2 percent by weight cobalt, 0 to 0.5 percent by weight manganese, 0 to 0.3 percent by weight molybdenum, 0 to 0.03 percent by weight phosphor, 0 to 0.03 percent by weight sulphur, 0 to 0.1 percent by weight nitrogen.

\* cited by examiner

## LOW COBALT HARD FACING ALLOY

## FIELD OF THE INVENTION

The present invention relates to steel alloys and particularly a chromium nickel silicon stainless steel alloy with low cobalt that may be suited for use in nuclear reactors, particularly in the components used in the steam generating plant of nuclear reactors.

## BACKGROUND OF THE INVENTION

Traditionally, cobalt-based alloys, including Stellite alloys, have been used for wear-based applications including, for example, in nuclear power applications. The alloys may be used to both form components or to provide hard-facing where harder or tougher material is applied to a base metal or substrate.

It is common for hard-facing to be applied to a new part during production to increase its wear resistance. Alternatively, hard-facing may be used to restore a worn surface. Extensive work in research has resulted in the development of a wide range of alloys and manufacturing procedures dependent on the properties and/or characteristics of the required alloy.

Within the nuclear industry the presence of cobalt within an alloy gives rise to the potential for the cobalt to activate within a neutron flux to result in the radioisotope cobalt-60 which has a long half-life. This makes the use of cobalt undesirable for alloys used in this industry. The cobalt may be released as the alloy wears through various processes, one of which is galling that is caused by adhesion between sliding surfaces caused by a combination of friction and adhesion between the surfaces, followed by slipping and tearing of crystal structure beneath the surface. This will generally leave some material stuck or even friction welded to the adjacent surface, whereas the galled material may appear gouged with balled-up or torn lumps of material stuck to its surface.

Replacements for Stellite have been developed by the industry with low or nil cobalt quantities. Exemplary alloys are detailed in the table below:

|                            | Alloy |         |         |         |          |           |     |     |         |
|----------------------------|-------|---------|---------|---------|----------|-----------|-----|-----|---------|
|                            | Cr    | C       | Nb      | Nb + Va | Ni       | Si        | Fe  | Co  | Ti      |
| GB2167088                  | 15-25 | 1-3     |         | 5-15    | 5-15     | 2.7-5.6   | Bal | Nil | Nil     |
| T5183                      | 19-22 | 1.8-2.2 | 6.5-8.0 |         | 8.5-10.5 | 4.5-5.25  | Bal | 0.2 | Trace   |
| U.S. Pat.<br>No. 5,660,939 | 19-22 | 1.7-2.0 | 8.0-9.0 |         | 8.5-10.5 | 5.25-5.75 | Bal | 0.2 | 0.3-0.7 |

In GB2167088 niobium is provided, but always with the presence of vanadium, which prevents the chromium from combining with the carbon and weakening the matrix. The vanadium also acts as a grain refiner within the wholly austenitic alloy that helps the keep the size of the grains within the alloy within an acceptable range.

The alloys of U.S. Pat. No. 5,660,939 modified the alloy of T5183 by the deliberate addition of titanium and by increasing the amounts of niobium and silicon. The controlled additions of titanium, niobium and silicon alter the structure of the steel to provide a duplex austenitic/ferritic microstructure which undergoes secondary hardening due to the formation of an iron silicon intermetallic phase.

Further hardening is achievable by hot isostatic pressing (HIPPING) of the stainless steel alloy when in powder form where secondary hardening occurs within the ferritic phase of the duplex microstructure.

The niobium provides a preferential carbide former over chromium, enabling high chromium levels to be maintained within the matrix so as to give good corrosion performance. Low cobalt based alloys, or cobalt alloy replacements, typically comprise significant quantities of carbide forming elements which can form alloys with hardness values in excess of 500 Hv. As with traditional Stellite alloys, the high levels of hardness observed can make machining difficult, resulting in poor mechanical properties for, for example, ductility, fracture toughness, impact resistance and workability. Additionally, the cost of using such alloys is high due to the need for special treatments and/or precision casting or other near net shape manufacturing methods to limit further machining.

Accordingly, it would therefore be advantageous to provide an alloy without the aforementioned disadvantages.

## SUMMARY OF THE INVENTION

The present invention accordingly provides, in a first aspect, an alloy consisting essentially of 19 to 22 percent by weight chromium, 8.5 to 10.5 percent by weight nickel, 5.25 to 5.75 percent by weight silicon, 0.25 to 2.0 percent by weight carbon, 4.0 to 10.5 percent by weight of a carbide former selected from the group consisting of molybdenum, tantalum, tungsten, zirconium and vanadium, 0.3 to 0.5 percent by weight titanium, 0.1 to 0.5 by weight percent nitrogen and the balance iron plus impurities.

The alloy may consist essentially of 19 to 22 percent by weight chromium, 8.5 to 10.5 percent by weight nickel, 5.25 to 5.75 percent by weight silicon, 0.25 to 2.0 percent by weight carbon, 4.0 to 10.5 percent by weight molybdenum, 0.3 to 0.5 percent by weight titanium, 0.1 to 0.5 by weight percent nitrogen and the balance iron plus impurities.

The alloy may consist essentially of 19 to 22 percent by weight chromium, 8.5 to 10.5 percent by weight nickel, 5.25 to 5.75 percent by weight silicon, 0.25 percent by weight carbon, 4.0 to 6.0 percent by weight molybdenum, 0.3 to 0.5 percent by weight titanium, 0.1 to 0.5 by weight percent nitrogen and the balance iron plus impurities.

percent by weight titanium, 0.1 to 0.5 by weight percent nitrogen and the balance iron plus impurities.

The alloy may consist essentially of 19 to 22 percent by weight chromium, 8.5 to 10.5 percent by weight nickel, 5.25 to 5.75 percent by weight silicon, 0.8 to 1.2 percent by weight carbon, 4.0 to 6.0 percent by weight molybdenum, 0.3 to 0.5 percent by weight titanium, 0.1 to 0.5 by weight percent nitrogen and the balance iron plus impurities.

The alloy may consist essentially of 19 to 22 percent by weight chromium, 8.5 to 10.5 percent by weight nickel, 5.25 to 5.75 percent by weight silicon, 1.7 to 2.0 percent by weight carbon, 8.5 to 10.5 percent by weight molybdenum, 0.3 to 0.5 percent by weight titanium, 0.1 to 0.5 by weight percent nitrogen and the balance iron plus impurities.



DETAILED DESCRIPTION OF THE  
PREFERRED EMBODIMENTS

The improved alloys described here have been developed having, in weight percent, 19 to 22 percent by weight chromium, 8.5 to 10.5 percent by weight nickel, 5.25 to 5.75 percent by weight silicon, 0.25 to 2.0 percent by weight carbon, 4.0 to 10.5 percent by weight of a carbide former selected from the group consisting of molybdenum, tantalum, tungsten, zirconium and vanadium, 0.3 to 0.5 percent by weight titanium, 0.1 to 0.5 by weight percent nitrogen and the balance iron plus impurities.

The impurities may be up to 0.2 wt % cobalt, up to 0.5 wt % manganese, up to 0.03 wt % phosphorus, up to 0.03 wt % sulphur and up to 0.1 wt % nitrogen. In the alloys which use titanium, tantalum, tungsten, zirconium or vanadium as the carbide former the alloy may contain an impurity of up to 0.3 wt % molybdenum

These compositions are similar to those proposed in U.S. Pat. No. 5,660,939 but there is a reduction in the niobium content and substitution with one or more carbide formers selected from the group consisting molybdenum, titanium, tantalum, tungsten, zirconium and vanadium.

Molybdenum is a carbide former which may be provided within the alloy in a quantity which further improves the properties of the alloy as it is provided in such a quantity that residual molybdenum following the formation of the carbides remains within the matrix and provides an improved pitting resistance.

In addition molybdenum carbide and tungsten carbide form at lower temperatures than niobium carbide and have a tendency to form molybdenum, or tungsten containing chromium carbides where the chromium content is in the range 19 to 22 by weight. Where niobium has been used as the carbide former it has been found that because it is a strong carbide former niobium carbides can form whilst atomising (or early on in casting if by that route) and grow which can then lead to nozzle blockages etc and hence low powder yield. Because molybdenum and tungsten have less affinity to form carbides than chromium the reaction with carbon provides molybdenum-containing chromium (Cr, Mo)C carbides rather than molybdenum carbides or tungsten-containing chromium (Cr, W)C carbides. In this way manufacturability of the alloy is maintained.

Exemplary alloy 1 consists essentially of 19 to 22 percent by weight chromium, 8.5 to 10.5 percent by weight nickel, 5.25 to 5.75 percent by weight silicon, 0.25 to 2.0 percent by weight carbon, 4.0 to 9.0 percent by weight titanium, 0.1 to 0.5 by weight percent nitrogen and the balance iron plus impurities.

Exemplary alloy 2 consists essentially of 19 to 22 percent by weight chromium, 8.5 to 10.5 percent by weight nickel, 5.25 to 6.0 percent by weight silicon, 1.7 to 2.0 percent by weight carbon, 8.0 to 9.0 percent by weight titanium, 0.1 to 0.5 by weight percent nitrogen and the balance iron plus impurities.

Exemplary alloy 3 consists essentially of 19 to 22 percent by weight chromium, 8.5 to 9.5 percent by weight nickel, 5.25 to 5.75 percent by weight silicon, 0.8 to 1.2 percent by weight carbon, 4.0 to 6.0 percent by weight titanium, 0.1 to 0.5 by weight percent nitrogen and the balance iron plus impurities.

Exemplary alloy 4 consists essentially of 19 to 22 percent by weight chromium, 8.5 to 10.5 percent by weight nickel, 5.25 to 5.75 percent by weight silicon, 0.25 percent by

weight carbon, 4.0 to 6.0 percent by weight titanium, 0.1 to 0.5 by weight percent nitrogen and the balance iron plus impurities.

Exemplary alloy 5 consists essentially of 19 to 22 percent by weight chromium, 8.5 to 10.5 percent by weight nickel, 5.25 to 5.75 percent by weight silicon, 0.25 to 2.0 percent by weight carbon, 4.0 to 9.0 percent by weight tantalum, 0.3 to 0.5 percent by weight titanium, 0.1 to 0.5 by weight percent nitrogen and the balance iron plus impurities.

Exemplary alloy 6 consists essentially of 19 to 22 percent by weight chromium, 8.5 to 10.5 percent by weight nickel, 5.25 to 6.0 percent by weight silicon, 1.7 to 2.0 percent by weight carbon, 8.0 to 9.0 percent by weight tantalum, 0.3 to 0.5 percent by weight titanium, 0.1 to 0.5 by weight percent nitrogen and the balance iron plus impurities.

Exemplary alloy 7 consists essentially of 19 to 22 percent by weight chromium, 8.5 to 9.5 percent by weight nickel, 5.25 to 5.75 percent by weight silicon, 0.8 to 1.2 percent by weight carbon, 4.0 to 6.0 percent by weight tantalum, 0.3 to 0.5 percent by weight titanium, 0.1 to 0.5 by weight percent nitrogen and the balance iron plus impurities.

Exemplary alloy 8 consists essentially of 19 to 22 percent by weight chromium, 8.5 to 10.5 percent by weight nickel, 5.25 to 5.75 percent by weight silicon, 0.25 percent by weight carbon, 4.0 to 6.0 percent by weight tantalum, 0.3 to 0.5 percent by weight titanium, 0.1 to 0.5 by weight percent nitrogen and the balance iron plus impurities.

Exemplary alloy 9 consists essentially of 19 to 22 percent by weight chromium, 8.5 to 10.5 percent by weight nickel, 5.25 to 5.75 percent by weight silicon, 0.25 to 2.0 percent by weight carbon, 4.0 to 9.0 percent by weight tungsten, 0.3 to 0.5 percent by weight titanium, 0.1 to 0.5 by weight percent nitrogen and the balance iron plus impurities.

Exemplary alloy 10 consists essentially of 19 to 22 percent by weight chromium, 8.5 to 10.5 percent by weight nickel, 5.25 to 6.0 percent by weight silicon, 1.7 to 2.0 percent by weight carbon, 8.0 to 9.0 percent by weight tungsten, 0.3 to 0.5 percent by weight titanium, 0.1 to 0.5 by weight percent nitrogen and the balance iron plus impurities.

Exemplary alloy 11 consists essentially of 19 to 22 percent by weight chromium, 8.5 to 9.5 percent by weight nickel, 5.25 to 5.75 percent by weight silicon, 0.8 to 1.2 percent by weight carbon, 4.0 to 6.0 percent by weight tungsten, 0.3 to 0.5 percent by weight titanium, 0.1 to 0.5 by weight percent nitrogen and the balance iron plus impurities.

Exemplary alloy 12 consists essentially of 19 to 22 percent by weight chromium, 8.5 to 10.5 percent by weight nickel, 5.25 to 5.75 percent by weight silicon, 0.25 percent by weight carbon, 4.0 to 6.0 percent by weight tungsten, 0.3 to 0.5 percent by weight titanium, 0.1 to 0.5 by weight percent nitrogen and the balance iron plus impurities.

Exemplary alloy 13 consists essentially of 19 to 22 percent by weight chromium, 8.5 to 10.5 percent by weight nickel, 5.25 to 5.75 percent by weight silicon, 0.25 to 2.0 percent by weight carbon, 4.0 to 9.0 percent by weight Zirconium, 0.3 to 0.5 percent by weight titanium, 0.1 to 0.5 by weight percent nitrogen and the balance iron plus impurities.

Exemplary alloy 14 consists essentially of 19 to 22 percent by weight chromium, 8.5 to 10.5 percent by weight nickel, 5.25 to 6.0 percent by weight silicon, 1.7 to 2.0 percent by weight carbon, 8.0 to 9.0 percent by weight Zirconium, 0.3 to 0.5 percent by weight titanium, 0.1 to 0.5 by weight percent nitrogen and the balance iron plus impurities.

Exemplary alloy 15 consists essentially of 19 to 22 percent by weight chromium, 8.5 to 9.5 percent by weight

nickel, 5.25 to 5.75 percent by weight silicon, 0.8 to 1.2 percent by weight carbon, 4.0 to 6.0 percent by weight Zirconium, 0.3 to 0.5 percent by weight titanium, 0.1 to 0.5 by weight percent nitrogen and the balance iron plus impurities.

Exemplary alloy 16 consists essentially of 19 to 22 percent by weight chromium, 8.5 to 10.5 percent by weight nickel, 5.25 to 5.75 percent by weight silicon, 0.25 percent by weight carbon, 4.0 to 6.0 percent by weight Zirconium, 0.3 to 0.5 percent by weight titanium, 0.1 to 0.5 by weight percent nitrogen and the balance iron plus impurities.

Exemplary alloy 17 consists essentially of 19 to 22 percent by weight chromium, 8.5 to 10.5 percent by weight nickel, 5.25 to 5.75 percent by weight silicon, 0.25 to 2.0 percent by weight carbon, 4.0 to 9.0 percent by weight vanadium, 0.3 to 0.5 percent by weight titanium, 0.1 to 0.5 by weight percent nitrogen and the balance iron plus impurities.

Exemplary alloy 18 consists essentially of 19 to 22 percent by weight chromium, 8.5 to 10.5 percent by weight nickel, 5.25 to 6.0 percent by weight silicon, 1.7 to 2.0 percent by weight carbon, 8.0 to 9.0 percent by weight vanadium, 0.3 to 0.5 percent by weight titanium, 0.1 to 0.5 by weight percent nitrogen and the balance iron plus impurities.

Exemplary alloy 19 consists essentially of 19 to 22 percent by weight chromium, 8.5 to 9.5 percent by weight nickel, 5.25 to 5.75 percent by weight silicon, 0.8 to 1.2 percent by weight carbon, 4.0 to 6.0 percent by weight vanadium, 0.3 to 0.5 percent by weight titanium, 0.1 to 0.5 by weight percent nitrogen and the balance iron plus impurities.

Exemplary alloy 20 consists essentially of 19 to 22 percent by weight chromium, 8.5 to 10.5 percent by weight nickel, 5.25 to 5.75 percent by weight silicon, 0.25 percent by weight carbon, 4.0 to 6.0 percent by weight vanadium, 0.3 to 0.5 percent by weight titanium, 0.1 to 0.5 by weight percent nitrogen and the balance iron plus impurities.

Exemplary alloy 21 consists essentially of 19 to 22 percent by weight chromium, 8.5 to 10.5 percent by weight nickel, 5.25 to 5.75 percent by weight silicon, 0.25 percent by weight carbon, 4.0 to 6.0 percent by weight molybdenum, 0.3 to 0.5 percent by weight titanium, 0.1 to 0.5 by weight percent nitrogen and the balance iron plus impurities.

Exemplary alloy 22 consists essentially of 19 to 22 percent by weight chromium, 8.5 to 10.5 percent by weight nickel, 5.25 to 5.75 percent by weight silicon, 0.8 to 1.2 percent by weight carbon, 4.0 to 6.0 percent by weight molybdenum, 0.3 to 0.5 percent by weight titanium, 0.1 to 0.5 by weight percent nitrogen and the balance iron plus impurities.

Exemplary alloy 23 consists essentially of 19 to 22 percent by weight chromium, 8.5 to 10.5 percent by weight nickel, 5.25 to 5.75 percent by weight silicon, 1.7 to 2.0 percent by weight carbon, 8.5 to 10.5 percent by weight molybdenum, 0.3 to 0.5 percent by weight titanium, 0.1 to 0.5 by weight percent nitrogen and the balance iron plus impurities.

In each of the above exemplary alloys impurities, which may be deliberately added, may be present. The impurities may be up to 0.2 wt % cobalt, up to 0.5 wt % manganese, up to 0.03 wt % phosphor, up to 0.03 wt % sulphur and up to 0.1 wt % nitrogen, up to 200ppm wt % oxygen. In the alloys which use titanium, tantalum, tungsten, zirconium or vanadium as the carbide former the alloy may contain an impurity of 0 to 0.3 wt % molybdenum

The new alloys have an acceptable galling resistance as carbides will still be formed, and the matrix continues to have a duplex austenitic/ferritic microstructure which undergoes secondary hardening due to the formation of an iron silicon intermetallic phase.

Further hardening is achievable by hot isostatic pressing (HIPPING) of the stainless steel alloy when in powder form where secondary hardening occurs within the ferritic phase of the duplex microstructure.

10 Although carbides continue to be formed the alloy has a resultant lower overall carbide caused, in part, by the weight percentage content of molybdenum and carbon giving an alloy with an acceptable hardness but greater ductility and toughness. This improvement in ductility opens up the range 15 of range of applications where consideration to shock events has to be considered as well as the overall wear resistance requirement.

The invention claimed is:

20 1. An alloy consisting essentially of 19 to 22 wt % chromium, 8.5 to 10.5 wt % nickel, 5.25 to 6.0 wt % silicon, 0.25 to 2.0 wt % carbon, 4.0 to 10.5 wt % of a carbide former selected from the group consisting of molybdenum, tantalum, tungsten, zirconium, and vanadium, 0.3 to 0.5 wt % titanium, 0.1 to 0.5 wt % nitrogen, and the balance being iron plus impurities.

25 2. The alloy according to claim 1, wherein the impurities consist of 0 to 0.2 wt % cobalt, 0 to 0.3 wt % molybdenum, 0 to 0.03 wt % phosphor, and 0 to 0.03 wt % sulphur, and 0 to 0.1 wt % nitrogen.

30 3. The alloy according to claim 1, wherein the carbide former is tantalum, and tantalum is 4.0 to 9.0 wt %.

35 4. The alloy according to claim 3, wherein the impurities consist of 0 to 0.2 wt % cobalt, 0 to 0.5 wt % manganese, 0 to 0.3 wt % molybdenum, 0 to 0.03 wt % phosphor, 0 to 0.03 wt % sulphur, and 0 to 0.1 wt % nitrogen.

40 5. The alloy according to claim 1, wherein the carbide former is tantalum, nickel is 8.5 to 9.5 wt %, silicon is 5.25 to 5.75 wt %, carbon is 0.8 to 1.2 wt %, and tantalum is 4.0 to 6.0 wt %.

45 6. The alloy according to claim 1, wherein the carbide former is tungsten, and tungsten is 4.0 to 9.0 wt %.

7. The alloy according to claim 6, wherein nickel is 8.5 to 9.5 wt %, silicon is 5.25 to 5.75 wt %, carbon is 0.8 to 1.2 wt %, and tungsten is 4.0 to 6.0 wt %.

50 8. The alloy according to claim 6, wherein the impurities consist of 0 to 0.2 wt % cobalt, 0 to 0.5 wt % manganese, 0 to 0.3 wt % molybdenum, 0 to 0.03 wt % phosphor, 0 to 0.03 wt % sulphur, and 0 to 0.1 wt % nitrogen.

9. The alloy according to claim 1, wherein the carbide former is zirconium, and zirconium is 4.0 to 9.0 wt %.

10. The alloy according to claim 9, wherein nickel is 8.5 to 9.5 wt %, silicon is 5.25 to 5.75 wt %, carbon is 0.8 to 1.2 wt %, and zirconium is 4.0 to 6.0 wt %.

55 11. The alloy according to claim 9, wherein the impurities consist of 0 to 0.2 wt % cobalt, 0 to 0.5 wt % manganese, 0 to 0.3 wt % molybdenum, 0 to 0.03 wt % phosphor, 0 to 0.03 wt % sulphur, and 0 to 0.1 wt % nitrogen.

12. The alloy according to claim 1, wherein the carbide former is vanadium, and vanadium is 4.0 to 9.0 wt %.

13. The alloy according to claim 12, wherein nickel is 8.5 to 9.5 wt %, silicon is 5.25 to 5.75 wt %, carbon is 0.8 to 1.2 wt %, and vanadium is 4.0 to 6.0 wt %.

60 14. The alloy according to claim 12, wherein the impurities consist of 0 to 0.2 wt % cobalt, 0 to 0.5 wt % manganese, 0 to 0.3 wt % molybdenum, 0 to 0.03 wt % phosphor, 0 to 0.03 wt % sulphur, and 0 to 0.1 wt % nitrogen.

**15.** An article comprising an alloy as claimed in claim 1.  
**16.** The alloy according to claim 1, wherein the alloy excludes niobium.

**17.** An alloy consisting essentially of 19 to 22 wt % chromium, 8.5 to 10.5 wt % nickel, 5.25 to 5.75 wt % silicon, 0.25 to 2.0 wt % carbon, 4.0 to 10.5 wt % molybdenum, 0.3 to 0.5 wt % titanium, 0.1 to 0.5 wt % nitrogen, and the balance being iron plus impurities. 5

**18.** The alloy according to claim 17, wherein carbon is 0.8 to 1.2 wt %, and molybdenum is 4.0 to 6.0 wt %. 10

**19.** The alloy according to claim 17, wherein carbon is 1.7 to 2.0 wt %, and molybdenum is 8.5 to 10.5 wt %.

**20.** The alloy according to claim 17, wherein the alloy excludes niobium.

\* \* \* \* \*

15